

# UNITED STATES PATENT OFFICE.

MILTON C. WHITAKER, OF NEW YORK, N. Y., ASSIGNOR TO U. S. INDUSTRIAL ALCOHOL CO., A CORPORATION OF WEST VIRGINIA.

## FUEL FOR INTERNAL-COMBUSTION ENGINES.

1,420,007.

Specification of Letters Patent. Patented June 20, 1922.

No Drawing.

Application filed November 12, 1919. Serial No. 337,397.

To all whom it may concern:

Be it known that I, MILTON C. WHITAKER, a citizen of the United States, residing at New York city, in the county of New York and State of New York, have invented a certain new and useful Improvement in Fuel for Internal Combustion Engines, of which the following is a specification.

My invention relates particularly to fuels 10 designed to be used in aeroplane motors, but is applicable for use in internal combustion motors of all kinds used in flying or for other purposes.

The object of my invention is to provide 15 a fuel which is especially adapted for use in aeroplanes, although it is also applicable for use in internal combustion engines in general.

It is necessary that fuels which are to be 20 used in aeroplane motors shall have great dependability, inasmuch as any uncertainty in the operation of the aeroplane, by reason of variability in the character of the fuel or failure of the fuel to perform its intended 25 work, may bring about disastrous consequences.

For this reason, it is desirable to avoid 30 using in such fuels large percentages of petroleum products, inasmuch as commercial petroleum products do not ordinarily have a constant composition, and are usually comprised of varying quantities of a number of different constituents.

It is, therefore, the object of my invention 35 to provide an aeroplane fuel avoiding these disadvantages and taking into account the circumstances above referred to.

Still a further object of my invention is 40 to provide fuels of the above character containing alcohol and a petroleum hydrocarbon blended by the use of benzol, and the constituents of which are chosen in such a manner as to obviate any tendency of the benzol to crystallize out or the constituents to 45 separate out within the range of atmospheric temperatures to which aeroplane motors are subjected at the varying altitudes in which aeroplanes operate.

Further objects of my invention will appear 50 from the detailed description thereof contained hereinafter.

While my invention is capable of being carried out in different ways, for the purpose of illustration I shall describe only certain ways of carrying out the same herein.

For example, a fuel made in accordance with my invention may be comprised of:

40 parts by volume of ethyl alcohol,  
30 parts by volume of benzol,  
30 parts by volume of ethyl acetate. 60

The percentages of the above constituents may vary to some extent, if desired. For example, the alcohol may vary from 35 to 50%, the benzol may vary from 25 to 35%, and the ethyl acetate may vary from 20 to 40%, although I have obtained the best results by the specific composition above given.

The ethyl alcohol in the above composition may be the ordinary alcohol having a 70 strength of 95%, but I may, if desired, use an alcohol having a greater strength, or even absolute alcohol.

By the use of the ethyl acetate I avoid 75 the necessity of using alcohol having a greater strength than 95%, as the ethyl acetate will prevent the benzol from crystallizing out at very low temperatures.

Instead of the ethyl alcohol, however, I 80 may use methyl alcohol or butyl alcohol, and instead of the benzol I may use toluol, and instead of the ethyl acetate I may use other esters such for example as methyl butyrate, ethyl butyrate, methyl acetate, butyl acetate or amyl acetate, all of which are volatile esters or still other esters could be used as for example, castor oil. 85

Aeroplane fuels made in the manner described above can be used with greatest reliability in the operation of aeroplanes, notwithstanding the varied atmospheric conditions to which aeroplane motors are subjected. 90

Nevertheless, all of these fuels are of such a nature that they may be readily used in internal combustion engines generally, whether used for operating aeroplanes or not. 95

While I have described my invention above in detail, I wish it to be understood that many changes may be made therein 100 without departing from the spirit thereof.

I claim:

1. A fuel comprising an alcohol, an aromatic hydrocarbon, and at least 20% of ethyl acetate. 105

2. A fuel comprising ethyl alcohol, an aromatic hydrocarbon, and at least 20% of ethyl acetate.

3. A fuel comprising an alcohol, benzol, and at least 20% of ethyl acetate. 110

4. A fuel comprising ethyl alcohol, benzol, and at least 20% of ethyl acetate.
5. A fuel comprising from 35% to 50% of an alcohol, from 25% to 35% of an aromatic hydrocarbon, and from 20% to 40% of an ester.
6. A fuel comprising from 35% to 50% of

ethyl alcohol, from 25% to 35% of benzol, and from 20% to 40% of ethyl acetate.

In testimony that I claim the foregoing,  
I have hereunto set my hand this 6th day of  
November, 1919.

MILTON C. WHITAKER.